

# UNITED STATES PATENT OFFICE.

CHARLES BESLAY, OF PARIS, FRANCE, ASSIGNOR TO EDWARD HECKSHER.

## IMPROVED PROCESS OF ELECTROPLATING IRON, STEEL, &c.

Specification forming part of Letters Patent No. 36,750, dated October 21, 1862.

*To all whom it may concern:*

Be it known that I, CHARLES BESLAY, of Paris, in the Empire of France, have invented certain new and useful Improvements in Electroplating Iron or Steel; and I hereby declare the following to be a full, clear, and exact description of the same.

My invention consists in a new mode of galvanizing metals—such as cast or wrought iron, steel, &c.—by an electro-chemical process in which the covering metal is applied indirectly—*i. e.*, by means of an intermediate metal—at the ordinary temperature (if above the freezing-point) and by using solutions not concentrated.

My invention therefore consists in the new application or adaptation of means and of electro-chemical manipulations already known—*i. e.*, in combining the several processes—so as to effect in an industrially practical manner galvanization of metals at the ordinary temperature, or what I term the “cold.”

In carrying out my invention I avail myself of the law of affinity which some metals in a greater or less degree have for other metals. For instance, it is well known that certain metals will readily combine with certain others by way of fusion, while others may with facility be deposited in a metallic state by electro-chemical process.

Now, iron forms with tin a series of alloys in which either the iron or the tin predominates. In the combination of these two metals the product or the alloy presents well-defined characteristics, constituting a homogeneous mass differing essentially from either of their constituents. Such will not be the result when iron is being combined with zinc or lead or copper; but since tin may be readily united with iron I first cover the iron with tin for the purpose of subsequently, through its medium, covering the iron with a metal with which it will not otherwise combine, the tin permitting such metal to be deposited upon it and intimately to unite therewith. The application of the intermediate metal covering to the galvanopating of iron is a very important feature of my invention. To explain, I suppose that iron is to be coated with zinc. The latter is well known to be a metal of little ductility, elasticity, and dilatability, whereas the former is a metal eminently ductile, elastic, and dilatable. The consequence is that the coating

would, by the molecular working of the iron, soon be destroyed, or at least become utterly inefficient as a preservative against oxidation, for which purpose it is mostly used. On the other hand, as the properties before mentioned increase in zinc in an inverse ratio with its thickness, it is desirable that the zinc coating of iron should be as thin as possible; but as a thin zinc covering could not efficiently protect the iron the intermediate layer of tin is used, whose ductility, elasticity, and dilatability excel those of iron and supply the deficiency in the thickness of the zinc coating. Thus a thin, elastic, and ductile zinc covering is used, which, combined with the tin having the same properties, offers the thickness of coating requisite for the proper protection of the iron.

The galvanization of common metals as heretofore attempted were simply laboratory experiments conducted on a very small scale, and which never resulted in a manufacturing process. In such experiments heat was resorted to as the easiest and readiest means to obtain from a given solution the metal to be deposited. The temperature in such solutions was allowed to reach from 25° to 60° and 80° centigrade—*i. e.*, from 90° to 150° and 200° Fahrenheit.

Reasons of economy—*i. e.*, the galvanization of common metals in a practical or industrial manner—render it important and necessary to operate at the ordinary temperature. For this purpose I use solutions of such nature as will allow of the work being carried out at the ordinary temperature without offering too great resistance to the galvanic current. In extremely cold weather the activity of the baths may be excited by increasing the electric force. I use for this purpose batteries of a peculiar construction having but one element capable of producing a continuous current sufficient at one operation to galvanize objects of one thousand pounds in about two cubic meters of solution. These batteries consist of a leaden vessel of about one and twenty one-hundredths meter in length by seventy-five one-hundredths of a meter in width and fifteen one-hundredths of a meter in depth. The bottom of this vessel is lined with a thin and movable copper sheet bent up at its edges. In this vessel I place, in the direction of its length, two wooden bars of from three one-hundredths to four one-hundredths of a meter in thickness, and upon these bars I put a thick sheet of zinc, to which

are secured or fixed the conductors. There is no diaphragm, and one battery thus made is equivalent to from twelve to fifteen elements of Daniell.

Heretofore it was deemed indispensable in electro-chemical applications to concentrate the solutions in order to precipitate metal upon metal. In the application of the electro-chemical process according to my invention it is of utmost importance to employ weak solutions or baths of feeble density. This I consider as a vital condition, without the fulfillment of which it is impossible to operate economically or in a manufacturing way. I use solutions of density not less than 3° according to Baumé's aerometer and not more than 6° Baumé. When during the operation, in consequence of evaporation, the solution becomes concentrated beyond 5° or 6° Baumé, I add water in the proportion of the water that shall have been evaporated. The diluted state of the solutions renders the tin, lead, and zinc salts less subject to alteration, while at the same time it puts them in a condition most favorable to be acted upon by electric currents. In the preparation of baths it was my endeavor to avoid the formation of stannates, zincates, plumbates, &c., they having a tendency in concentrated solutions to precipitate in a crystalline state, of becoming less and less soluble, of creating gelatinous deposits, and of then presenting great-

est resistance to electro-chemical decomposition; and I have found that it is easier to maintain in a soluble state subsalts, whether alkaline or acid, if used in solutions not concentrated. I prefer to use the metastannates and the protocyanides of tin, either separately or combined with each other or combined with analogous substances of zinc or lead base; the sub or proto sulphates and the subacetates of zinc, &c., combined together—in general, all double combinations in which the subsalts of the metallic base enter in but feeble proportions.

Having thus described my improvements in the galvanization of iron, steel, &c., and the manner in which the same are or may be carried into effect, I claim as invention—

The electro-chemical galvanization of iron, steel, &c., by combining with an intermediate metal, applied in the manner herein described, the method of effecting the galvanization proper at ordinary temperature in solutions not concentrated, substantially as herein set forth.

In testimony whereof I have signed my name to this specification before two subscribing witnesses.

CH. BESLAY.

Witnesses:

GEO. HUTTON,  
JAMES W. BROOKS.